

## UNITED STATES PATENT OFFICE

2,518,372

## ALKYL SUBSTITUTED THIOPHENE SULFONIC ACID SALTS AS DETERGENTS IN MINERAL OIL COMPOSITIONS

Orland M. Reiff and Harry J. Andress, Jr., Woodbury, N. J., assignors to Socony-Vacuum Oil Company, Incorporated, a corporation of New York

No Drawing. Application November 20, 1946,  
Serial No. 711,212

5 Claims. (Cl. 252—33)

1

This invention relates to improved mineral oil compositions and to new chemical compounds for improving them. More specifically, this invention relates to mineral oil compositions containing salts of alkylated thiophene sulphonates in concentrations sufficient to improve the properties thereof and to the salts of alkylated thiophene sulphonates per se.

A number of oil-soluble detergents of the type of metal soaps, phenylates and alkylates have been proposed and used as crank case oils to dissolve or disperse the sludge and prevent lacquer deposits and stuck piston rings. Unfortunately, however, the great majority of these substances increase the rate of oxidation and their presence results in an increased concentration of acidic oxidation products in the oil. Increased quantities of these acidic oxidation products in the oil create, in turn, an even more serious difficulty for they attack and corrode alloy bearings commonly employed in internal combustion engines. Alloys composed of copper-lead, silver-cadmium, nickel-cadmium, etc., are widely used and are subject to attack by the acidic oxidation products formed in the oil.

Certain anti-corrosion agents which have no detergent properties have been added to lubricating oils in order to counteract the corrosive effect of the oxidation products of the oil. Although many of the detergents and the anti-corrosion agents which have been previously mentioned perform their individual functions in lubricating oils, the two separate chemicals do not cooperate to produce a satisfactory anti-corrosion and detergent action when used together.

The function of a corrosion inhibitor is to cover the bearing surfaces and other corrodable parts of the engine with a passivating film that prevents corrosion of the metal by the organic acids and other corrosive products of the oil. A detergent, as its name implies, operates to remove adhering materials from the metal parts of the engine and thus produce a clean metal surface. Consequently, heretofore known mixtures of a detergent with a corrosion inhibitor have proven to be ineffective over any extended period of time, since the detergent action of the sludge inhibitor tends to remove the corrosion inhibitor from the metal surface, thus rendering it ineffective for the purpose intended.

In accordance with the present invention, a series of new compounds have been discovered, which compounds act in a highly satisfactory manner as detergents and which at the same time improve the pour point of the oil and the viscosity

2

index of the oil. Furthermore, it has been discovered that these new compounds can be used in combination with anti-corrosion or stabilizing agents, without impairing the effectiveness of either agent.

## THE OIL BASE

The basic materials to which the improving agents of this invention are to be added may be generally described as mineral lubricating oils of the type normally used in internal combustion engines. Such oils are generally produced from petroleum but may be produced synthetically from other sources. It is contemplated that the principles of this invention may be applied to lighter petroleum products such as gasoline and kerosene or to heavier petroleum products of the nature of petroleum gear lubricants, petroleum jellies and petroleum waxes.

## DETERGENT

The detergent or cleaning agent of this invention consists of one or a mixture of salts of alkylated thiophene sulphonates. In most cases these will be metal salts of alkylated thiophene sulphonates and when the metal is polyvalent the salt may be either a neutral salt containing several alkylated thiophene sulphonate radicals per molecule, or an alkaline salt containing fewer radicals of alkylated thiophene sulphonate per molecule than are necessary to satisfy the valence of the metal, the remaining valences of metal being satisfied by carbonate or hydroxy radicals, or the like. Preferred, are the alkaline earth metal salts, examples of which are the barium, calcium and magnesium salts. For the purpose of this specification, magnesium is included in the alkaline earth metal group.

The term "thiophene" as used in this specification, may be expanded to include "thiophene-like" materials, such as thionaphthene. Derivatives of these materials similar to the derivatives of thiophene, which will be specifically disclosed, will function in a similar manner.

The thiophene radical of the new compounds is alkylated in at least one position and the alkyl substituent is preferably a long chain aliphatic hydrocarbon group containing at least ten carbon atoms, such for example as the alkyl radical obtained from paraffin wax. Although there is no known upper limit to the number of carbon atoms in the alkyl chain, it is preferred that there be not more than thirty. There are three places in thiophene sulphonate where the thiophene nucleus can be substituted and any one or all three of these places may have sub-

stituents. There appears to be no limit as to what these substituents can be, except that it is necessary to have at least one alkyl substituent and it is preferred, mainly for reasons of oil solubility, to have at least one, relatively long chain, alkyl substituent. The compounds will function, however, for their intended purpose, even though the alkyl substituent is relatively short.

Concentrations in oil of from about 0.5% to about 10% of the new detergent agent are contemplated in this invention, but concentrations of from 2% to 5% have been found most satisfactory and hence are preferred.

#### STABILIZING AGENT

Although any known stabilizing or anti-oxidation agent may be used in combination with the new detergent agent in oil, particularly desirable results have been achieved by the use of a small amount of an oil-soluble, phosphorus-sulphur-containing reaction product of a dicyclic terpene and a phosphorus sulphide. Such products may be prepared in accordance with United States Patent application, Serial No. 482,482, filed April 9, 1943, now abandoned, by Fuller et al.

The following specific examples will illustrate the manner by which the detergent agents may be prepared.

#### EXAMPLE I

A paraffin wax having an average of about 24 carbon atoms in the molecule and an ASTM melting point of about 126° F. was chlorinated at about 100° C. with gaseous chlorine until the weight of the wax had increased by about 14%. The resultant chlorwax was then blown with nitrogen to remove any occluded hydrogen chloride or chlorine.

610 g. of the thus prepared chlorwax was stirred with 140 g. of powdered calcium oxide for about 6 hours at about 255-265° C. and then filtered through a layer of absorptive clay, to give a product which will be referred to as unsaturated wax or wax olefin.

280 g. of the unsaturated wax were mixed with 100 g. of thiophene and about 150 g. of a powdered synthetic silica-alumina gel catalyst containing 7 to 15% alumina. The mixture was placed in an autoclave and heated to about 200° C. for 4 hours. A pressure drop of about 175 lbs. per square inch was observed. The reaction mixture was filtered through a layer of absorptive clay and topped at 175° C. under 10 mm. mercury of pressure to give a product that is apparently a monowax alkylated thiophene.

246 g. of the above wax alkylated thiophene were blended with 246 g. of an SAE-10 grade motor oil and stirred at room temperature with 44.4 g. of chlorsulphonic acid for about 1 hour. The temperature was then slowly raised to about 100° C. and 50 g. of barium hydroxide octahydrate were added along with about 200 g. of butyl alcohol, to facilitate removal of the water formed during the reaction. The reaction mixture was then heated to about 175° C. and filtered through a layer of absorptive clay. All traces of water and butanol were removed by distillation at about 175° C. under 10 mm. of mercury pressure. The product, a barium salt of wax alkylated thiophene sulphonate, showed, upon analysis, about 4.9% barium and about 2.8% sulphur, in the 1:1 oil blend.

#### EXAMPLE II

1194 g. of 14% chlorwax, prepared as described in Example I, were mixed with 179 g. of dibutyl-

thiophene and heated to about 80° C. and 36 g. of anhydrous aluminum chloride then added. The reaction mixture was stirred for 3 hours at about 125° C. and then for 1 hour at about 165° C. The mixture was then cooled to about 100° C. and a large excess of water added to break up the aluminum chloride complex. The resultant mixture was filtered through a layer of absorptive clay and the product water-washed to free it of hydrogen chloride and aluminum hydroxide. Thereafter it was topped at 175° C. under 10 mm. of mercury pressure to give a wax alkylated dibutylthiophene.

To 547 g. of this product was added 91 g. of chlorsulphonic acid at room temperature, and the mixture was slowly heated to about 100° C. for about 1 hour. The mixture was then cooled to about 75° C. and 123 g. of barium hydroxide octahydrate was added along with 200 g. of butyl alcohol. This mixture was heated to about 165° C., filtered through a layer of absorptive clay and topped at 175° C. under 10 mm. of mercury pressure. The resultant product, a barium salt of wax substituted dibutyl thiophene sulphonate, was shown by analysis to contain about 3.1% barium and about 5.2% sulphur.

#### EXAMPLE III

1004 g. of 14% chlorwax, prepared as described in Example I, was mixed with 230 g. of a mixture of alpha and beta methyl thiophene and heated to about 75-80° C. 30 g. of anhydrous aluminum chloride was added, the temperature raised to about 110° C. and held for about 3/4 hour. The mixture was further heated to about 175° C. for 1 hour to complete the reaction. The aluminum chloride complex was destroyed by adding an excess of water to the mixture at about 100° C. and the resultant mixture was filtered through a layer of absorptive clay. All traces of hydrogen chloride and aluminum hydroxide were removed by thorough water-washing as before. The finished product was obtained by topping the resultant mixture at about 175° C. under 10 mm. mercury of pressure. This product was apparently a diwax alkylated methylthiophene.

300 g. of this product was blended with 300 g. of SAE-10 grade mineral oil, and the mixture heated to 50 to 60° C. and 66.3 g. of chlorsulphonic acid then added. The temperature was thereafter raised slowly to about 100° C. and held for 1 hour, then cooled to about 75° C. and 90 g. of barium hydroxide octahydrate and 200 g. of butyl alcohol added and the temperature again raised to about 165° C. for 1 hour. As before, the mixture was filtered through a layer of absorptive clay and topped at 175° C. under 10 mm. pressure to give the finished product. This product is apparently a barium salt of diwax methylthiophene sulphonate showing upon analysis 4.3% barium and 2.9% sulphur in the approximately 1:1 mineral oil blend.

#### EXAMPLE IV

65 As an example of an antioxidant or stabilizing agent, that may advantageously be used in combination with the detergent agents described above, a pinene-phosphorus pentasulphide reaction product was prepared in accordance with the disclosure of United States Patent application, Serial No. 482,482, filed April 9, 1943, by Fuller et al.

According to this procedure a mixture of 800 g. of pinene and 800 g. of a motor oil (SUV 45 seconds at 210° F.) was heated to 105° C. and

## 5

while stirring, 326.4 g. of phosphorus pentasulphide were added slowly, the temperature increasing to 115° C., because of the exothermic nature of the reaction. The temperature was then raised to 150° C. and maintained there for 1 hour. After partial cooling, and the addition of 32 g. of absorptive clay, the mixture was filtered. The filtrate was topped at 150° C. at 5 mm. mercury of pressure, leaving a clear, viscous oil containing 12.5% sulphur and 5.11% phosphorus, by weight.

## EXAMPLE V

In order to illustrate the effectiveness of the new sulphonates in depressing the pour point of mineral oils, various percentages of the sulphonates made in accordance with Examples II and III were blended with a mineral oil having a Saybolt Universal viscosity of 67 seconds at 210° F. The following table shows the results:

Table I

| Improving Agent    | Concentration, Per Cent by Weight | ASTM Pour Point, °F. |
|--------------------|-----------------------------------|----------------------|
| None               | 0                                 | +20                  |
| Product of Ex. II  | 1                                 | -15                  |
| Do                 | 1/2                               | -15                  |
| Product of Ex. III | 1/2                               | -30                  |
| Do                 | 1/2                               | -25                  |

## EXAMPLE VI

The viscosity index improvement that can be effected by the use of the new sulphonates is illustrated by the following table which shows the results of adding various concentrations of the products of Examples II and III to a mineral oil similar to that used in Example V.

Table II

| Improving Agent        | Conc., Percent by Weight | Kinematic Visc. at 100° F. | Kinematic Visc. at 210° F. | Viscosity Index |
|------------------------|--------------------------|----------------------------|----------------------------|-----------------|
| None                   | 0                        | 30.55                      | 4.82                       | 78.5            |
| Product of Example II  | 1                        | 35.9                       | 5.44                       | 92.7            |
| Product of Example III | 1                        | 36.8                       | 5.65                       | 99.7            |

## EXAMPLE VII

Lauson oxidation stability tests were conducted on certain blends containing both the sulphonates of this invention and the stabilizing agent described in Example IV, to determine the effectiveness of the stabilizing agent in the presence of the new sulphonates.

The Lauson oxidation stability test is conducted in a Lauson single cylinder, four cycle, liquid cooled gasoline engine with jet lubrication.

A 1/2 gallon sample of the product to be tested is added at the beginning of the run and no oil is added during the test. 100% straight run gasoline plus 2.5 cc. of tetraethyl lead is used as the fuel and the test consists of operating the engine for 36 hours under standard conditions, and thereafter determining the neutralization number and kinematic viscosity at 210° F. of the oil.

During the test, the oil temperature is 280° F., the jacket temperature of the engine is 212° F., the speed of the engine is 1815 R. P. M., the throttle setting is 1/4, and the fuel-air ratio is 13:1.

In the test, the results of which are recorded in Table III, a mineral lubricating oil having a

## 6

Saybolt viscosity of 45 seconds at 210° F. was used as the base oil. To this oil were added the materials indicated.

Table III

| Improving Agent                                              | Neutralization No. | Kinematic Viscosity at 210° F. |
|--------------------------------------------------------------|--------------------|--------------------------------|
| None                                                         | 10.0               | 12.71                          |
| 4% of Product of Example I and 1/4% of Product of Example IV | 1.1                | 5.98                           |
| 4% of Product of Example III and 1/4% of Example IV          | 1.4                | 6.17                           |

## EXAMPLE VIII

To further indicate the effectiveness of the new mineral oil compositions in internal combustion engine lubrication operation tests known as

20 C. F. R. ring sticker tests, were conducted using a motor oil of 120 seconds Saybolt Universal viscosity at 210° F. without any addition agents and with the addition of 4% of the sulphonate of Example III and 1/4% of the stabilizing agent of Example IV.

The C. F. R. ring sticker test is conducted in the C. F. R. fuel test engine modified for lubricant evaluation. This is a single cylinder, liquid cooled engine equipped to give controlled oil flow

30 to the crankpin. A one gallon sample of the product to be tested is added at the beginning of the run and no oil is added during the test. Using 91 octane no. aviation gasoline, the test is run for 28 hours with the oil temperature at 175° F., the jacket temperature at 390° F. and a speed of 1200 R. P. M. The following items are reported: Actual number of degrees of ring sticking for all 5 rings; deposits in ring grooves of 3 oil rings; and total weight of deposits inside and

40 outside of piston exclusive of lead deposits from gasoline.

Table IV.—Ring condition

| Improving Agent                                              | Degrees Stuck | Percent Slot Filled |     |     |     |    | Carbon Deposit | Neutralization No. |      |
|--------------------------------------------------------------|---------------|---------------------|-----|-----|-----|----|----------------|--------------------|------|
|                                                              |               | 1                   | 2   | 3   | 4   | 5  |                |                    |      |
|                                                              |               | 3                   | 4   | 5   | 6   | 7  |                |                    |      |
| None                                                         | 360           | 360                 | 360 | 360 | 360 | 60 | 70             | 70                 | 14.0 |
| 4% of Product of Example III + 1/4% of Product of Example IV | 0             | 0                   | 0   | 0   | 0   | 5  | 5              | 0                  | 6.1  |

## EXAMPLE IX

Indicative of the fact that the new detergent agents are effective even in the presence of stabilizing agents are the results of a series of Lauson detergency tests.

60 The Lauson detergency test consists in operating a single cylinder, four cycle, liquid cooled, jet lubrication, Lauson gasoline engine for 30 hours, using 1/2 gallon of the oil to be tested and then checking the oil for neutralization number and the engine for cleanliness. The engine cleanliness is rated on a scale of 0 to 100, 100 representing a perfectly clean engine.

During the test, the engine is operated on 100% straight run gasoline plus 2.5 cc. of tetraethyl lead, no oil is added, the oil temperature is 225° F., the jacket temperature 350° F., and the speed of the engine 1830 R. P. M. The throttle setting is 1/2, and the fuel-air ratio is 13:1.

In the following tests, a motor oil of 67 seconds

Saybolt Universal viscosity at 210° F. was used as the base oil.

Table V

| Improving Agent                                              | Clean-<br>liness<br>Rating | Neutral-<br>ization<br>No. |
|--------------------------------------------------------------|----------------------------|----------------------------|
| None                                                         | 51                         | 4.0                        |
| 5% of Product of Example II + 1/2% of Product of Example IV  | 84                         | 1.0                        |
| 4% of Product of Example III + 3/4% of Product of Example IV | 72                         | 0.5                        |

It is contemplated by this invention that the new alkyl substituted thiophene-like sulphonate salts will be incorporated in lubricating oil compositions in amounts sufficient to improve the characteristics of the oils. It is further contemplated that such oils may contain a stabilizing agent such as described in Example IV or any other stabilizing agent, pour point depressant, extreme pressure lubrication improving agent, viscosity improving agent, or other agent that it is found desirable to incorporate. It is also contemplated by this invention that the new alkyl substituted thiophene-like sulphonate salts may be marketed per se, or in more concentrated admixtures with oil, which admixtures are adapted to be added to further quantities of oil to improve its characteristics.

What is claimed is:

1. A mineral lubricating oil composition comprising a mineral oil and a minor proportion, sufficient to improve the detergent properties of the oil, of an alkyl substituted thiophene alkaline earth metal sulphonate salt in which the

alkyl substituent contains a carbon chain about ten to about thirty carbon atoms in length.

2. A mineral lubricating oil composition comprising a mineral oil and a minor proportion, sufficient to improve the detergent properties of the oil, of a petroleum wax substituted thiophene alkaline earth metal sulphonate salt.

3. A mineral lubricating oil composition comprising a mineral oil and a minor proportion, sufficient to improve the detergent properties of the oil, of a petroleum wax substituted thiophene sulphonate barium salt.

4. A mineral lubricating oil composition comprising a mineral oil and between about .05% and about 10% of a petroleum wax substituted thiophene sulphonate barium salt.

5. A mineral lubricating oil composition comprising a mineral oil and between about 2% and about 5% of a di-petroleum wax substituted sulphonate barium salt.

ORLAND M. REIFF.  
HARRY J. ANDRESS, JR.

## REFERENCES CITED

25 The following references are of record in the file of this patent:

## UNITED STATES PATENTS

Number Name Date  
30 2,197,835 Reiff ----- Apr. 23, 1940

## OTHER REFERENCES

Beilstein's Handbuch der Organischen Chemie,  
4th ed. vol. XVIII, p. 570.  
35 Whitmore: Organic Chemistry, 1937, p. 893.